

## 1

3,284,276

COATED CELLOPHANE ARTICLE AND PROCESS  
FOR OBTAINING THE SAME

Morris B. Berenbaum, Levittown, Pa., Rolf F. Foerster, Hamilton Square, N.J., Riad H. Gobran and David C. Guth, Levittown, Pa., Ronald F. Snyder, Bordentown, N.J., and Theodore F. Wells III, Morrisville, and Arthur J. Yu, Levittown, Pa., assignors to Thiokol Chemical Corporation, Bristol, Pa., a corporation of Delaware  
No Drawing. Filed Nov. 6, 1962, Ser. No. 235,839

9 Claims. (Cl. 161—184)

The present invention relates to a novel composition and process for the coating of cellulosic materials such as cellophane, wood and paper, including cardboard, cylinder board and paper board. More particularly the present invention relates to a novel solution system containing a polyepoxide and a copolymer of vinylidene chloride and an  $\alpha,\beta$ -unsaturated carboxylic acid or an anhydride of such acids which may be used to coat cellulosic substrates.

This is a continuation in part, of application S.N. 215,290, entitled "Cellophane Coating Composition and Process," filed in the name of Morris B. Berenbaum et. al. on Aug. 17, 1962, now abandoned.

An object of the present invention is to provide a composition with which coatings can be readily and economically imparted to cellulosic substrates, and in particular those cellulosic substrates which are customarily employed as flexible films in the packaging industry such as cellophane or the various types of paper such as kraft paper and glassine.

Another object of the present invention is to provide a coating composition which will allow the imparting of coatings to cellulosic substrates which are clear and have excellent heat sealing and solvent and grease resistance as well as good adhesive (to substrate) and vapor impermeability properties.

A further object of this invention is to provide a process whereby cellulosic substrates may be readily coated with such compositions.

A still further object of the present invention is to provide for the preparation of fire resistant, flexible laminates made of cellulosic substrates.

Cellophane, wood and paper are all cellulosic in nature, wood being a natural product and paper being processed from wood pulp. Cellophane is a form of regenerated (from viscose) cellulose in transparent sheet form. Cellophane and paper are used as packaging materials for many applications, including, the packaging of food items, cigarettes and other tobacco products, items of apparel, etc. For the cellophane to be flexible enough for such applications it should contain a certain quantity of water. This amount of water, moreover, must be sealed in the cellophane by coating the cellophane with a coating having good moisture impermeability properties. The coating also prevents the cellophane, in rolled form from blocking during storage. If the coated cellophane or paper is to come in contact with grease or oil, moreover, such as in various food packaging applications, the coating must also be grease and oil resistant. Polymeric cellophane coating materials of this type include vinylidene chloride/acrylonitrile copolymers, vinylidene chloride/alkyl acrylate copolymers and vinylidene  $\alpha,\beta$ -unsaturated carboxylic acid copolymers such as are disclosed in U.S.

## 2

2,334,236; 2,748,027; 2,762,720; 2,805,963; 2,819,984; 3,034,929; 3,037,868; 3,039,986 and Great Britain 889,564. In order to coat the cellophane with these type polymers, however, it is usually necessary to first treat the cellophane with an anchoring agent whereby a useful degree of adhesion between the film and the cellophane base sheet may be obtained. Even when these anchoring agents are used with many of the commercially available cellophane coating materials, however, the degree of adhesion obtained between the base sheet and the film coating is inadequate for many applications. The solvent and grease resistant properties of the coating obtained with these polymers, moreover, is limited to that afforded by the polymers themselves and there has been no way known to the art, to date, to vary or improve such properties for cellophane coating applications. There are many applications also which require that wood substrates used therein be protected with coatings which are resistant to penetration or attack by moisture, grease, solvents and the like.

It has now been unexpectedly found, according to the present invention, that cellulosic substrates may be readily coated with a clear coating which has good adhesion to the cellulosic substrate as well as excellent heat sealing and solvent and grease resistant properties and good vapor impermeability properties if the substrate is first coated with a solution containing:

(a) At least one polyepoxide compound, and  
(b) At least one copolymer of vinylidene chloride and at least one  $\alpha,\beta$ -unsaturated carboxylic acid or an anhydride or such acids and the polyepoxide is then reacted with the copolymer to form a crosslinked reaction product concurrent with and/or subsequent to the removal of the solvent medium.

To our knowledge, the present invention represents the first successful attempt to those in the art to use an epoxy crosslinked, vinylidene chloride/ $\alpha,\beta$ -unsaturated carboxylic acid copolymer for coating cellulosic substrates and in particular, cellophane, although epoxy crosslinked carboxyl group containing copolymers have been used extensively for other purposes: i.e., U.S. 2,604,457; 2,604,463; 2,604,464; 2,965,602; 2,662,870; 2,759,901; 2,798,861; 2,969,602; 2,985,616 and 3,027,357; Canadian 534,001; 534,261 and 569,430 and Great Britain 681,031 and 896,821.

The vinylidene chloride copolymers of the present invention are relatively low molecular weight particulate materials which contain about 75 to 95 and preferably about 85 mol percent of vinylidene chloride and about 5 to 25 and preferably about 15 mol percent of at least one unsaturated  $\alpha,\beta$ -carboxylic acid such as acrylic, methacrylic, itaconic and crotonic acids or anhydrides of such acids. They are random copolymers which are soluble in selected solvents such as tetrahydrofuran, ethyl acetate, acetone, methyl ethyl ketone, methyl isobutyl ketone, dimethyl formamide and dioxane and cosolvent systems such as those containing at least 50% by volume of tetrahydrofuran and at least one solvent diluent such as toluene and methylene chloride.

The copolymers are preferably formed by means of a free radical polymerization reaction using about 0.1 to 4% by weight of a catalyst such as azobisisobutyronitrile or benzoyl peroxide. The reaction is preferably conducted in solution in a solvent such as hexane, methylisobutylketone, methyl ethyl ketone, acetone or 50/50

(by volume) acetone/toluene. The polymerization reaction may also be conducted using suspension and emulsion polymerization techniques. The copolymers produced should preferably be freed of heavy metal contaminants, such as iron, for stability purposes.

The polyepoxides which may be used in the novel composites and processes of the present invention are those which contain an average of more than one epoxide



group per molecule and which are soluble in the desired solvent. Generally speaking, all the polyepoxide materials commercially available today may be used in the composition and processes of the present invention, whether they are solid or liquid materials. The polyepoxy materials which can be cured with the above described copolymers are preferably those materials which have an average epoxy functionality of more than one and preferably they are materials which contain an average of at least approximately two epoxide groups per molecule of the polyepoxy material. The position of the epoxide groups in the polyepoxy material is not critical. For instance, if the polyepoxy material is essentially linear in structure the epoxide groups may be in a terminal position or they may be positioned intermediately and/or randomly along the linear structure. Polyepoxy materials which may be cured with the above defined copolymers include the following types of materials:

(1) Essentially linear type such as



homopolymers and copolymers of glycidyl acrylate and preferably a copolymer of vinylidene chloride and glycidyl acrylate and the epoxidized polybutadiene materials such as those which have an epoxide functionality of four or more and which are sold by Food Machinery Corporation under the designation "Oxiron" resins (i.e., "Oxiron 2000," "Oxiron 2001," and "Oxiron 2002").

(2) Bisphenol A/epichlorohydrin type which are aromatic in nature and which include those sold by the Thiokol Chemical Corporation under the trademark designation "Tipox" (i.e., "Tipox A"; "Tipox B"; "Tipox C") those sold by the Shell Chemical Company under the designation "Epon" resins, i.e., "Epon 828" and those sold by Union Carbide Chemicals Company under the designation "Bakelite ERL" resins.

(3) Cycloaliphatic type which includes those sold by Union Carbide Chemicals Company under the designation "Unox" resins (i.e., "Unox 206" which is epoxy ethyl-3,4-epoxy cyclohexane, "Unox 201" which is 3,4-epoxy-6 - methylcyclohexylmethyl - 3,4-epoxy-6-methylcyclohexanecarboxylate, "Unox 221" which is 3,4-epoxy-cyclohexylmethyl - 3,4 - epoxy cyclohexane carboxylate and "Unox 289" which is bis(3,4-epoxy-6-methylcyclohexylmethyl) adipate.

(4) Resorcinol diglycidyl ether type which includes those sold by Koppers Chemical Corporation under the designation "Kopoxite" resins (i.e., "Kopoxite 159").

(5) Epoxy novolak type (alkyl novolak resins) which is a phenolic/epoxy type system and which includes the resins sold by Dow Chemical Corporation under the designation "Dow Epoxy Novolak 438" or "DEN 438-EK 85" which contains 85% of the resin and 15% methyl ethyl ketone as a solvent and the resins sold by Koppers Chemical Corporation under the designation "KER" resins (i.e., "KER 357A" and "KER 955A").

(6) Epoxidized fatty acid resins including the Epoxol materials sold by Swift and Company such as "Epoxol 9-5" (epoxidized linseed oil) and "Epoxol 7-4" (epoxidized soy bean oil); the "Flexol" resins sold by Union Carbide Chemical Company, such as "Flexol EP8" (2-ethyl hexyl epoxy tallate). "Flexol EPO" (epoxidized soy bean oil) and "Flexol TPO" (epoxidized soy bean oil) and "Paraplex G62" (epoxidized soy bean oil) sold by Rohm & Haas.

(7) Epoxidized silicone oil types such as that marketed by Dow Corning under the trade name "Epoxy Silicone QZ", e.g., Epoxy Silicone QZ8-0914.

For the purpose of obtaining the approval of the Food and Drug Administration of the Department of Health, Education, and Welfare for the cellophane coating compositions of the present invention in food packaging applications, the epoxidized fatty acid type polyepoxides are the preferred of such compounds. The Unox resins, and in particular the Unox 201 and Unox 289 type resins are preferred of the polyepoxide compounds for room temperature curing applications. The higher the functionality of the polyepoxide compound, the tighter the cure that is obtained usually, all other factors remaining the same and for some applications such higher functional polyepoxide materials are preferred. The use of glycidyl acrylate copolymers, such as, a copolymer of vinylidene chloride and glycidyl acrylate is preferred in those applications where a less plasticized coating is desired for better coating surface properties.

0 "Tixop B" resin is preferred for those coatings requiring good clarity and heat sealing properties.

The polyepoxide/copolymer solution systems of the present invention offer unique handling and processing advantages to the trade. They are essentially one package curing systems and are stable upon storage for extended periods of time. Their solids content can be readily varied to meet the need for various types of applications. Those in the trade seem to prefer a solution having a solids content of about 15 to 35% by weight. By solids content it is meant, the percent by weight of those components of the solutions which are not solvents, even though one or more of the other components, such as the polyepoxide materials, may be liquid under normal conditions. The solution nature of these systems also provides for a facile incorporation therein of adjuvant materials such as pigments, dyes, delustrants, plasticizers, waxes, fillers, stabilizers, etc., when desired. Solvents which may be used in the preparation of the coating solution of the present invention include methyl ethyl ketone, tetrahydrofuran, methyl isobutyl ketone and solvent mixtures containing no more than about 75% toluene and the remainder tetrahydrofuran, methyl ethyl ketone and/or ethyl acetate. The preferred solvents are methyl ethyl ketone or a mixture of toluene with methyl ethyl ketone or ethyl acetate.

In coating cellulosic substrates according to the present invention, a solution containing the polyepoxide and the copolymer is applied to the substrate on one or more faces or sides thereof as desired, so as to provide each face or side of the substrate being coated with a film which is at least about 0.05 and is preferably about 0.1 to 1 mil thick after the removal of the solvent therefrom. The coatings may be applied by any of the commonly used dipping, brushing, roller coating, etc., techniques known to the art. The viscosity of the coating may be varied to suit the manner of application by adjusting the solids content of the coating solution. The solvent is then removed preferably at elevated temperatures under forced draft conditions. The temperatures employed with cellophane substrates is preferably about 125° to 150° C. and with glassine substrates temperatures as high as about 200° to 210° C. may be used. At these temperatures the removal of the solvent and the crosslinking of the copolymer and the polyepoxide can be accomplished, simultaneously in a matter of seconds. At 150° C., the removal of the sol-

vent and the crosslinking reaction could take up to 10 to 15 seconds and if conducted at room temperature the procedures could take up to twenty four hours with those polyepoxides which will crosslink with the copolymer at room temperature. The crosslinking reaction involves the reaction of the carboxyl groups of the copolymer with the epoxy groups of the polyepoxide. About 0.01 to 2.5 and preferably about 0.1 to 1.0 mol of epoxide moieties should be provided per mol of carboxyl moieties to insure adequate crosslinking sites. Catalysts such as tertiary amines,  $\text{BF}_3$  and  $\text{BF}_3$  complexes may be used to facilitate the crosslinking reaction when using certain of the polyepoxide materials such as the epichlorohydrin/bisphenol A type. Useful products may be obtained with these polyepoxides, however, without the use of such catalysts. The use of increased amounts of the longer chained (aliphatic/fatty acid) type polyepoxides tends to produce tacky and self-adhering coatings which are particularly useful for some packaging applications.

The coatings produced according to the present invention are normally crosslinked and/or chain extended into a very high molecular weight form with the application of heat, yet they retain very excellent heat sealing properties. If a coating material does not have heat sealing properties, its utility in the field of packaging coatings would be sharply curtailed since heat sealability of the coated packaging material is a necessary prerequisite to its universal utility as a wrapping material.

The coatings prepared according to the present invention have much better solvent, grease and scratch resistant properties and are much more resistant to the passage of moisture therethrough than the coatings presently available for coating cellulosic substrates largely due to the crosslinked and/or chain extended nature of the coatings of the present invention. There are, to our knowledge, no crosslinked plastic based coatings for cellulosic substrates commercially available today, all the cellulosic substrate coating materials presently available to the art being thermoplastic in nature.

The coatings produced by the present invention also provide a much better adhesion of the coating to the cellulosic substrate than has hitherto been thought possible to those in the art. The coatings of the present invention may be applied to the substrate and used therewith for a number of applications without having the coating anchored to the cellulosic substrate with the aid of the so-called anchoring agents. These anchoring agents are apparently not needed in the preparation of the cellulosic substrates coated according to the present invention for use in many applications where anchored coatings were thought to be indispensable. It is thought that a reaction takes place between some of the pendant carboxyl groups of the copolymers of the present invention and various of the reactive groups of the cellulosic substrate whereby this unusual adherence of the coating to the substrate is af-

5 fected. For use under extreme conditions the adherence of the coatings of the present invention to the cellulosic substrate can be supplemented by use of commonly employed anchoring agents such as melamine/formaldehyde and urea/formaldehyde resins.

10 The carboxylic acid moieties supply the copolymers of the present invention, for the most part, with its solubility properties in addition to supplying the copolymer with the carboxyl groups needed to subsequently anchor the coating to the cellulosic substrate and crosslink with the epoxy groups of the polyepoxide compounds. The solubility of the copolymers can also be varied, if desired, by varying the molecular weight of the copolymer. The vinylidene chloride units of the copolymer help to supply the needed vapor impermeability and grease resistant properties to the crosslinked coating. The polyepoxide materials supply the epoxide groups needed to crosslink the copolymer via its carboxyl groups. It is the crosslinked and/or chain extended nature of the coatings of the present invention which provides its excellent solvent resistant properties. The polyepoxide materials also probably imparts adhesive and plasticized properties to the cured coating which is particularly useful in a flexible packaging application. The liquid polyepoxides also act as cosolvents for the copolymer. It can be readily seen, therefore, that the novel coating compositions of the present invention provide those in the art with a versatile coating system, the components and/or amounts of the components of which can be readily changed so as to provide for the needs of a vast variety of end use coating applications.

15 The following examples are merely illustrative of the present invention and are not intended as a limitation upon the scope thereof.

#### EXAMPLES 1-15

20 Among the vinylidene chloride copolymers which may be used to form part of the curable compositions of the present invention are those of vinylidene chloride ( $\text{VCl}_2$ ) and acrylic acid (AA). Curable copolymers made from those monomers were prepared by solution polymerization as illustrated in Tables I and II below. They represent a wide range of compositions, produced using several solvent systems, e.g., solvent A=methylisobutylketone; solvent B=acetone; solvent C=1:1 vol./vol. mixture of acetone and toluene, solvent D=methylethyl ketone and several free radical polymerization initiators, e.g., initiator A=azobis-butyronitrile; initiator B=benzoyl peroxide, under various polymerization conditions of temperature and time, to provide reactive copolymers at various percentages of conversion of the monomers. In preparing these copolymers, the respective initiators were dissolved in the solvent used and the monomers were then added to the initiator solution. The reactions were conducted under nitrogen in a sealed reaction vessel under autogenous pressure.

Table I

| Ex. | Charge            |       | Charge Mol Percent, $\text{VCl}_2/\text{AA}$ | Initiator |      | Solvent |      |
|-----|-------------------|-------|----------------------------------------------|-----------|------|---------|------|
|     | $\text{VCl}_2$ g. | AA g. |                                              | In grams  | Type | In ml.  | Type |
| 1   | 63                | 25    | 65/35                                        | 2         | A    | 150     | A    |
| 2   | 73                | 17    | 75/25                                        | 2         | A    | 150     | A    |
| 3   | 155               | 29.6  | 80/20                                        | 4         | A    | 240     | A    |
| 4   | 78                | 14    | 80/20                                        | 2         | A    | 150     | A    |
| 5   | 78                | 14.4  | 80/20                                        | 2         | A    | 150     | A    |
| 6   | 3,220             | 496   | 83/17                                        | 80        | A    | 6,000   | D    |
| 7   | 161               | 25    | 83/17                                        | 4         | A    | 300     | A    |
| 8   | 161               | 24.5  | 83/17                                        | 4         | A    | 300     | C    |
| 9   | 161               | 24.5  | 83/17                                        | 4         | A    | 300     | D    |
| 10  | 161               | 24.5  | 83/17                                        | 6         | B    | 300     | C    |
| 11  | 161               | 24.5  | 83/17                                        | 6         | B    | 300     | D    |
| 12  | 83                | 10.8  | 85/15                                        | 2         | A    | 150     | A    |
| 13  | 83                | 10.8  | 85/15                                        | 2         | A    | 150     | A    |
| 14  | 171               | 17    | 88/12                                        | 4         | A    | 300     | A    |
| 15  | 87                | 7.2   | 90/10                                        | 2         | A    | 150     | A    |

Table II

| Example | Reaction   |             |                     | Resin Product                    |                          |
|---------|------------|-------------|---------------------|----------------------------------|--------------------------|
|         | Time, Hrs. | Temp., ° C. | Conversion, Percent | Mol Percent VCl <sub>2</sub> /AA | G. eq. COOH/100 g. Resin |
| 1       | 5          | 60          | 57                  | 72/28                            | 0.32                     |
| 2       | 4          | 60          | 79/21               | 0.22                             |                          |
| 3       | 16         | 65          | 85                  | 82/18                            | 0.19                     |
| 4       | 4          | 60          | 32                  | 83/17                            | 0.18                     |
| 5       | 17         | 60          | 85                  | 83/17                            | 0.19                     |
| 6       | 6          | 65          | 61                  | 83.9/16.1                        | 0.173                    |
| 7       | 3          | 65          | 53                  | 84/16                            | 0.17                     |
| 8       | 5          | 65          | 63                  | 84/16                            | 0.17                     |
| 9       | 5          | 65          | 61                  | 85/15                            | 0.161                    |
| 10      | 5          | 65          | 33                  | 85/15                            | 0.161                    |
| 11      | 5          | 65          | 38                  | 86/14                            | 0.149                    |
| 12      | 4          | 60          | 33                  | 87/13                            | 0.13                     |
| 13      | 1          | 85          | 55                  | 87/13                            | 0.14                     |
| 14      | 3          | 65          | 55                  | 90/10                            | 0.11                     |
| 15      | 1          | 85          | 56                  | 91/9                             | 0.10                     |

The resin products obtained were soluble in the pot product mixture. They were separated therefrom by precipitation from solution through the addition of ice and water to the pot products, and by a subsequent

sealable and were about 0.2 to 0.3 mil thick. The formulations use in these examples and water vapor permeability values of the coating thus obtained are shown in the following table.

Table III

| Example                                                                   | 16    | 17    | 18    | 19    | 20    | 21    | 22    | 23    | 24    | 25     | 26     | 27    | 28    |
|---------------------------------------------------------------------------|-------|-------|-------|-------|-------|-------|-------|-------|-------|--------|--------|-------|-------|
| Formulation (parts by weight, grams):                                     |       |       |       |       |       |       |       |       |       |        |        |       |       |
| VCl <sub>2</sub> /AA Copolymer                                            | 100   | 100   | 100   | 100   | 100   | 100   | 100   | 100   | 100   | 100    | 100    | 100   | 100   |
| Flexol EP8 epoxy resin                                                    | 26.2  | 100   | 100   | 100   | 100   | 100   | 100   | 100   | 100   | 100    | 100    | 100   | 100   |
| Flexol EPO epoxy resin                                                    |       | 17.3  |       |       |       |       |       |       |       |        |        |       |       |
| Flexol JPO epoxy resin                                                    |       |       | 17.3  |       |       |       |       |       |       |        |        |       |       |
| Epoxol 7-4 epoxy resin                                                    |       |       |       | 24.1  |       |       |       |       |       |        |        |       |       |
| Epoxol 9-5 epoxy resin                                                    |       |       |       |       | 14.9  |       |       |       |       |        |        |       |       |
| Unox 201 epoxy resin                                                      |       |       |       |       |       | 13.1  | 13.1  | 2.62  |       |        |        |       |       |
| Unox 289 epoxy resin                                                      |       |       |       |       |       |       |       |       | 18.0  | 8.97   | 26.9   |       |       |
| Paraplex G62 epoxy resin                                                  |       |       |       |       |       |       |       |       |       |        |        | 20.9  |       |
| Tipox B epoxy resin                                                       |       |       |       |       |       |       |       |       |       |        |        |       | 16.0  |
| Toluene                                                                   | 358   | 333   | 333   | 352   | 326   |       | 321   | 290   | 335   | 309    | 360    | 343   | 329   |
| Ethyl Acetate                                                             | 358   | 333   | 333   | 352   | 326   |       | 321   | 290   | 335   | 309    | 360    | 343   | 329   |
| Methyl Ethyl Ketone                                                       |       |       |       |       |       | 642   |       |       |       |        |        |       |       |
| COOH/epoxy ratio                                                          | 0.5/1 | 0.5/1 | 0.5/1 | 0.5/1 | 0.5/1 | 0.5/1 | 0.5/1 | 0.1/1 | 0.5/1 | 0.25/1 | 0.75/1 | 0.5/1 | 0.5/1 |
| Specific permeability of cellophane and coating (milligrams/square inch): |       |       |       |       |       |       |       |       |       |        |        |       |       |
| High (of 5 samples)                                                       | 373   | 73.6  | 163   | 241   | 101.9 | 27.8  | 50.1  | 62.5  | 54.5  | 269    | 70.6   | 617.0 | 60.3  |
| Low                                                                       | 167   | 38.6  | 52.8  | 108   | 28.9  | 24.4  | 30.7  | 13.8  | 30.4  | 26.9   | 22.7   | 134.8 | 31.5  |
| Average                                                                   | 288   | 56.5  | 90.0  | 175   | 47    | 25.7  | 41.4  | 35.6  | 41.2  | 95.5   | 39.0   | 317.3 | 44.1  |
| Specific permeability of coating only (milligrams/square inch):           |       |       |       |       |       |       |       |       |       |        |        |       |       |
| High                                                                      | 76.5  | 10.9  | 25.4  | 40.0  | 18.8  | 4.65  | 7.93  | 15.7  | 10.2  | 51.0   | 14.9   | 121.0 | 12.7  |
| Low                                                                       | 34.2  | 5.7   | 8.22  | 17.9  | 5.34  | 4.08  | 4.87  | 3.48  | 5.68  | 5.09   | 4.78   | 26.4  | 6.6   |
| Average                                                                   | 58.8  | 8.4   | 14.1  | 28.9  | 6.9   | 43.1  | 6.6   | 8.94  | 7.71  | 18.09  | 8.23   | 62.2  | 9.3   |

filtering, fragmentation, washing with water, further filtering and a subsequent drying of the solids copolymers under vacuum at about 50° C. The copolymers, when dried, are white, particulate materials. Using osmometric techniques it has been found that copolymers produced in this manner have number average molecular weights of about 10,000±2,000.

#### EXAMPLES 16-28

Cellophane was coated in thirteen different runs (referred to as Examples 16-28) according to the present invention, with various solutions, each of which having about a 15% solids content and composed of an 84.5/15.5 VCl<sub>2</sub>/AA copolymer produced as in Examples 1 to 15 and different polyepoxides and solvents as disclosed below. The cellophane was coated on one side using a reverse roll coater commonly employed for coating flexible substrates. The (cellophane delivery) web roll speed was 7.9 feet/minute. After passing over the metering roll, speed was 20 feet/minute and the windup roll speed was 7.9 feet/minute. After passing over the metering roll, the solution coated cellophane was passed through two heating zones (ovens), each of which was 12 feet long. The temperature of the first was 200° F. and that of the second was 250° F. The solvent was removed and the curing of the coating occurred substantially in these heating zones. The coatings thereby obtained were heat

50 The water vapor permeability values obtained in the above examples indicate that cellophane coated according to the present invention may be used commercially in a variety of packaging applications. Specific permeabilities are given in milligrams of water vapor passing through a one mil film per square inch of exposed area in 24 hours at 72° F. over one molal NaCl solution. The values were calculated for the combination of cellophane base sheet and coating as well as for the coating above.

60 Specific permeability  

$$= \frac{\text{weight gain in mg}}{\text{exposed area}} \times \frac{\text{thickness of film in mils}}{\text{exposed area}}$$

65 (ASTM E96-53T). Coatings having similar properties may also be prepared using other VCl<sub>2</sub>/AA Copolymers prepared as in Examples 1 to 15.

#### EXAMPLE 29

70 A vinylidene chloride/glycidyl acrylate (VCl<sub>2</sub>/GA) copolymer was prepared by polymerizing 165 g. of vinylidene chloride and 38 grams of glycidyl acrylate in 300 ml. of methyl ethyl ketone at 65° C. using 5 grams of azobisisobutyronitrile as a polymerization initiator. The reaction took 2 hours. The copolymer was recovered in 46.5% yield as a white, solid, particulate material by

precipitating it from the polymerization solution into two volumes of 80/20 by volume methanol/water and then washing the precipitated copolymer with the same non-solvent mixture. The copolymer was then dried and clear solutions of it in tetrahydrofuran at 20% solids indicated that very little, if any, crosslinking of the  $VCl_2/AA$  copolymer had occurred. The copolymer had a molecular weight of about  $10,000 \pm 2,000$  and contained 88 mol percent vinylidene chloride and 12 v. mol percent glycidyl acrylate.

### EXAMPLES 30-32

Cellophane was coated in three different runs (Examples 30-32) according to the present invention with three different solutions, each of which having about a 15% solids content and composed of an 84.5/15.5  $VCl_2/AA$  copolymer, tetrahydrofuran as the solvent and, as the polyepoxide component, and 88/12 mol percent ratio  $VCl_2/GA$  copolymer produced as in Example 29.

The cellophane was hand coated (on one side) with these solutions and the coatings were cured for 20 seconds at  $300^{\circ} F$ . The resulting coatings were heat sealable and were about 0.2 to 0.3 mil thick. The formulations used for these coatings and the water vapor permeabilities of the resulting coated cellophane materials are shown below.

| Example                                                                              | 30   | 31   | 32   |
|--------------------------------------------------------------------------------------|------|------|------|
| Formulation (parts by weight, grams):                                                |      |      |      |
| $VCl/AA$                                                                             | 5    | 5    | 5    |
| $VCl/GA$                                                                             | 3.45 | 5.18 | 6.9  |
| Tetrahydrofuran                                                                      | 48   | 57.7 | 67.5 |
| Epoxide/COOH ratio (by equivalents)                                                  | 0.5  | 0.75 | 1.00 |
| Specific permeabilities (milligrams/square inch), cellophane base sheet and coating: |      |      |      |
| High                                                                                 | 32.8 | 20.4 | 20.1 |
| Low                                                                                  | 13.1 | 11.3 | 11.4 |
| Average                                                                              | 16.9 | 15.1 | 16.3 |
| Coating alone:                                                                       |      |      |      |
| High                                                                                 | 3.27 | 3.33 | 3.72 |
| Low                                                                                  | 1.98 | 1.85 | 2.12 |
| Average                                                                              | 2.55 | 2.46 | 3.03 |

The results indicate that the coatings of the present invention have good, reproducible, water vapor permeability properties even when applied with crude coating techniques.

### EXAMPLE 33

Stock polyepoxide solutions 1 to 18 were prepared so as to contain 15% solids using Oxiron 2000 resin in Cellosolve acetate (solution 1); diacetone alcohol (solution 2), and toluene (solution 3); Tipox B resin in methyl isobutyl ketone (solution 4), chloroform (solution 5) and Solvesso 150/Cellosolve acetate (in 9/1 wt./wt. ratio) (solution 6); Unox 221 resin in acetone (solution 7), cyclohexane (solution 8) and methanol (solution 9); Kkopoxite 159 resin in butyl Cellosolve acetate (solution 10), trichloroethylene (solution 11) and ethanol (solution 12); KER 357-A resin in dimethyl formamide (solution 13), methylene chloride (solution 14) and xylol (solution 15) and Epoxol 9-5 resin in dioxane (solution 16), benzene (solution 17) and butyl acetate (solution 18).

Further, two stock solution of a  $VCl_2/AA$  copolymer were prepared: Solution I contained 15% solids in tetrahydrofuran and Solution II contained 15% solids in a 1:1 mixture by weight of methyl ethyl ketone and ethyl acetate. The copolymer contained vinylidene chloride and acrylic acid in an 84.5/15.5 mol ratio and was made as in Examples 1 to 15.

Coating solutions A to R were then prepared by mixing together various weights of the stock polyepoxide and  $VCl_2/AA$  copolymer solutions according to the schedule in Table IV, below, to produce solutions containing epoxide/carboxyl ratios in equivalents of 2, 1 and 0.5.

10  
Table IV

|    | Coating Solution Formed | Poly-epoxide Solution Used | Grams of Poly-epoxide Solution Used | VCl <sub>2</sub> /AA Solution Used | Grams of VCl <sub>2</sub> /AA Solution Used | Ratio Epoxide/Carboxyl Equivalents in the Coating Solutions |
|----|-------------------------|----------------------------|-------------------------------------|------------------------------------|---------------------------------------------|-------------------------------------------------------------|
| 5  | A                       | 1                          | 60                                  | I                                  | 100                                         | 2                                                           |
|    | B                       | 2                          | 30                                  | I                                  | 100                                         | 1                                                           |
|    | C                       | 3                          | 15                                  | I                                  | 100                                         | 0.5                                                         |
| 10 | D                       | 4                          | 64                                  | I                                  | 100                                         | 2                                                           |
|    | E                       | 5                          | 32                                  | I                                  | 100                                         | 1                                                           |
|    | F                       | 6                          | 16                                  | I                                  | 100                                         | 0.5                                                         |
|    | G                       | 7                          | 44.6                                | I                                  | 100                                         | 2                                                           |
|    | H                       | 8                          | 22.3                                | I                                  | 100                                         | 1                                                           |
|    | I                       | 9                          | 11.2                                | I                                  | 100                                         | 0.5                                                         |
| 15 | J                       | 10                         | 43                                  | I                                  | 100                                         | 2                                                           |
|    | K                       | 11                         | 21.5                                | II                                 | 100                                         | 1                                                           |
|    | L                       | 12                         | 10.75                               | II                                 | 100                                         | 0.5                                                         |
|    | M                       | 13                         | 66.6                                | II                                 | 100                                         | 2                                                           |
|    | N                       | 14                         | 33.3                                | II                                 | 100                                         | 1                                                           |
|    | O                       | 15                         | 16.7                                | II                                 | 100                                         | 0.5                                                         |
| 20 | P                       | 16                         | 5.9                                 | II                                 | 100                                         | 2                                                           |
|    | Q                       | 17                         | 29.5                                | II                                 | 100                                         | 1                                                           |
|    | R                       | 18                         | 15                                  | II                                 | 100                                         | 0.5                                                         |

Various cellulosic substrates, namely 35 lb. unwaxed kraft type paper and uncoated wooden medical-type tongue depressor sticks were dip coated with each of 25 coating solutions A to R and cured at  $83^{\circ} F$ ., for about 16 hours.

Adhesion of the coatings to the substrates was then tested. The coatings were scored with a razor to form a diamond shaped cut. Pressure sensitive type (cellophane-type) was pressed onto the cut areas and surrounding coated surface, and then quickly removed by pulling. No delamination occurred as a result of this test, all coatings were securely bonded to their respective substrates.

### EXAMPLE 34

Two stock solutions were prepared: Solution Y being 15% solids of an 84.5/15.5 mol ratio  $VCl_2/AA$  copolymer prepared as in Examples 1-15 in tetrahydrofuran, and solution Z being 45 g. of the epoxidized silicone oil Epoxy Silicone QZ8-0914 in 25 g. of toluene (this oil has an epoxide equivalent of 185). A coating solution was then prepared to contain a 1/1 ratio of equivalents of epoxy/carboxyl by mixing together 31 g. of solution Z with 100 g. of solution Y. Various 45 cellulosic substrates i.e., 35 lb. unwaxed kraft paper and uncoated wooden tongue depressor sticks were then dip coated with this coating solution at room temperature and the resulting coatings were cured in air for about 15 minutes at  $78^{\circ} F$ . to produce coated objects wherein 50 the adhesion of the cured coating to the substrate was excellent in each case.

### EXAMPLE 35

Paper materials are often used as inexpensive gasketing, 55 the useful work-life thereof being determined by the length of time in which these materials retain their flexibility and impermeability. Wood used in contact with water also has a useful working life dependent upon its resistance to the absorption of water. In this example 60 samples of paper and wood were used as substrates, said substrates being normally highly water absorbent. The paper used was laboratory filter paper, and the wood used was an uncoated medical tongue depressor. One half of the paper and wood were dip coated with a 40% solids 65 coating solution comprising 20 parts by weight (p.b.w.) of a vinylidene chloride/acrylic acid copolymer having a  $VCl_2/AA$  mol percent of 84.5/15.5 and prepared as in Examples 1-15 and 3 p.b.w. of the polyepoxide resin Epoxol 9-5 in 34.5 p.b.w. of the solvent system tetrahydrofuran/toluene (1/1 wt./wt.). The solution had a ratio in equivalents of epoxide/carboxyl of 0.5/1. The 70 coatings were permitted to air cure for 8-10 hours at about  $80^{\circ} F$ . to produce thereby cellulosic structures being in part uncoated and in part coated with a cured coating. The coated portion of the paper structure was 75

still quite flexible and when both portions, the coated and uncoated portions, were immersed in a stream of water the uncoated portion quickly became wet and readily absorbed water whereas the coated portion did not absorb water, the drops of water readily rolling off the coated surface. Similar observations were made with regard to the coated and uncoated portions of the wooden depressor stick.

## EXAMPLE 36

Glassine paper, which is a heat and pressure treated nonporous smooth and translucent paper material, is often used in the packaging of food stuffs and other substances. In this example, glassine paper was used as the substrate material and was coated with various polyepoxide-vinylidene chloride ( $VCl_2$ ) acrylic acid (AA) copolymer coating solutions. The  $VCl_2$ /AA copolymer had a mol ratio of 84.5/15.5  $VCl_2$ /AA and was prepared as in Examples 1-15. Solutions were prepared according to the recipes given in the table below to form mixtures having a 25% solids content in a 1/1 by weight solvent system of methyl ethyl ketone (MEK)/ethyl acetate (EA). The solutions were applied to one surface side of squares of glassine paper so as to form wet films 2-3 mils thick thereon. The coated glassine paper was air dried for about 1 min. at about 80° F., and then was subjected to 300° F. temperatures for 5 minutes to produce thereby cellulosic structures in which the cured organic coating obtained was smooth, bubble-free and found to be strongly adherent to the glassine paper substrate. The pressure sensitive tape test was used to determine the qualities of adhesion of the cured coating to the paper substrate. In this test pressure-sensitive cellophane tape was firmly pressed onto the coated surface of the structure in two places. The first piece of tape was rapidly delaminated and the second piece slowly delaminated from the coated surface. In no instance were any of the cured coatings removed or loosened from the glassine paper substrate.

p.s.i. pressure for 75 min. to produce, in one instance a nine ply laminate designated Laminate A. In another instance another 9 ply laminate, Laminate B, was produced by heating nine coated squares, placed one atop the other, to a temperature of 300° F. under an impressed pressure of 1000 p.s.i. also for 75 min. The laminates obtained showed excellent resistance to attack by trichloroethylene vapor this being an important property of laminates useful in the making of printed circuit components. The solvent vapor resistance test used involves exposing a 2" x 3" piece of laminate to an atmosphere of trichloroethylene vapors at a pressure of 760 mm. Hg for a 5 minute interval, drying the laminate at ambient temperatures for 24 hours and then inspecting the laminate for leechout of the laminating resin.

The recipe and laminating conditions used, and the properties obtained for laminates A and B are listed in the table below.

|                                             |        | Laminate A | Laminate B |
|---------------------------------------------|--------|------------|------------|
| Recipe of Varnish, p.b.w.:                  |        |            |            |
| $VCl_2$ /AA copolymer                       | 100    | 100        | 100        |
| Tipox A resin                               | 80     | 80         | 80         |
| $BF_3$ MEA                                  | 3      | 3          | 3          |
| Cure Conditions:                            |        |            |            |
| Drying time, min.                           | 1      | 1          | 1          |
| Drying temperature, °F.                     | 212    | 212        | 212        |
| Cure time, min.                             | 75     | 75         | 75         |
| Cure temperature, °F.                       | 275    | 300        | 300        |
| Cure pressure, p.s.i.                       | 1,000  | 1,000      | 1,000      |
| Number of plies                             | 9      | 9          | 9          |
| Properties of Laminates:                    |        |            |            |
| Thickness, inches                           | 0.058  | 0.064      | 0.064      |
| Specific gravity                            | 1.46   | 1.44       | 1.44       |
| Flexural strength, p.s.i.                   | 19,000 | 18,500     | 18,500     |
| Tensile strength, p.s.i.                    | 8,300  | 6,300      | 6,300      |
| Percent elongation                          | 4      | 4          | 4          |
| Rockwell hardness                           | 78     | 78         | 78         |
| Vapor Resistance, 5 min., Trichloroethylene | (1)    | (1)        | (1)        |

<sup>1</sup> Excellent.

Table V

| Recipe in p.b.w.:                      | 100 | 100 | 100   | 100   | 100   | 100   | 100   | 100   | 100   | 100   | 100   | 100   | 100   |
|----------------------------------------|-----|-----|-------|-------|-------|-------|-------|-------|-------|-------|-------|-------|-------|
| $VCl_2$ /AA                            | 100 | 100 | 100   | 100   | 100   | 100   | 100   | 100   | 100   | 100   | 100   | 100   | 100   |
| 1/1 MEK/EA                             | 390 | 417 | 364.5 | 367.2 | 389.1 | 393.6 | 389.1 | 345   | 358.5 | 332.4 | 333.6 | 344.7 | 346.8 |
| Epoxol 9-5 resin                       | 30  |     |       |       |       |       |       | 15    |       |       |       |       |       |
| Epoxol 7-5 resin                       |     | 39  |       |       |       |       |       |       | 19.5  |       |       |       |       |
| Kopoxite 159 resin                     |     |     | 21.5  |       |       |       |       |       | 10.8  |       |       |       |       |
| Uiron 221 resin                        |     |     |       | 22.4  |       |       |       |       |       | 11.2  |       |       |       |
| D.E.N. 438 resin                       |     |     |       |       | 29.7  |       |       |       |       |       | 14.9  |       |       |
| Tipox A resin                          |     |     |       |       |       | 31.2  |       |       |       |       |       | 15.6  |       |
| Oxiron 2000 resin                      |     |     |       |       |       |       | 29.7  |       |       |       |       |       | 14.9  |
| Ratio of Equivalents, Epoxide/Carboxyl | 1/1 | 1/1 | 1/1   | 1/1   | 1/1   | 1/1   | 1/1   | 0.5/1 | 0.5/1 | 0.5/1 | 0.5/1 | 0.5/1 | 0.5/1 |
| Percent Solids                         | 25  | 25  | 25    | 25    | 25    | 25    | 25    | 25    | 25    | 25    | 25    | 25    | 25    |

## EXAMPLE 37

Paper laminates having superior resistance to solvent vapors were produced through the use of vinylidene chloride/acrylic acid copolymer polyepoxide varnishes as the laminating means.

In this example an impregnating solution, commonly known as "varnish" in the laminating arts, was prepared by dissolving 100 p.b.w. of an 84.5/15.5 mol percent ratio vinylidene chloride/acrylic acid ( $VCl_2$ /AA) copolymer produced as in Example 1-15 80 p.b.w. of the polyepoxide resin Tipox A and 3 p.b.w. of  $BF_3$ -monoethylamine ( $BF_3$ MEA) cure catalyst in 123 p.b.w. of methyl ethyl ketone. This varnish was then used to coat 16" x 16" squares of 0.010" cotton linters paper that had previously been treated with Bakelite's water soluble phenolic varnish 3913 at a 14.5-17% resin content; which treatment is a standard precoat or "1st pass" treatment in the laminating arts for use with paper and laminating resins. The coated squares of treated paper were then heated to 212° F. for about 1 min. under infra-red radiation to remove the solvent and allow the coating to become dry and tack-free. Nine of the thus coated squares were then placed one atop the other, thence into a laminating press, and there heated to 275° F. under 1000

55  
60  
65  
70  
75

The chemical and solvent resistance of laminates A and B was further tested through immersion in 30%  $H_2SO_4$ , carbon tetrachloride and n-heptane for 24 hours at about 73° F. No changes in the laminates were observed, under these test conditions.

We claim:

- As an article of manufacture a cellophane substrate coated on at least one surface thereof with the reaction product of
  - at least one copolymer essentially consisting of about 75 to 95 mol percent of vinylidene chloride and about 5 to 25 mol percent of at least one acid material selected from the group consisting of  $\alpha,\beta$ -unsaturated, aliphatic carboxylic acids and their anhydrides, and
  - at least one polyepoxide in an amount such as to provide about 0.01 to 2.5 mols of epoxide groups per mol of carboxyl groups present in said copolymer.
- An article as in claim 1 in which said polyepoxide contains an average of more than one epoxide group per molecule.
- An article as in claim 1 in which said acid material is acrylic acid.
- An article as in claim 1 in which said copolymer contains about 85 mol percent of vinylidene chloride.

5. A process for coating a cellophane substrate comprising applying to at least one surface of said substrate a solution containing

(A) at least one copolymer essentially consisting of about 75 to 95 mol percent of vinylidene chloride and about 5 to 25 mol percent of at least one acid material selected from the group consisting of  $\alpha,\beta$ -unsaturated, aliphatic carboxylic acids and their anhydrides, and

(B) at least one polyepoxide in an amount such as to provide about 0.01 to 2.5 mols of epoxide groups per mol of carboxyl groups present in said copolymer, removing the solvent medium from said solution, and crosslinking said copolymer with said polyepoxide whereby said crosslinked copolymer forms a coating on said substrate.

6. A process as in claim 5 in which the removal of said solvent medium and the crosslinking of said copolymer occurs substantially simultaneously.

7. A process as in claim 6 in which said solvent medium is removed at elevated temperatures.

8. A process as in claim 5 in which at least one face of

10

15

20

said substrate is provided with a coating having a thickness of at least about 0.05 mils.

9. An article as in claim 1 wherein said polyepoxide is selected from the group consisting of an epoxidized fatty acid, a polymer containing glycidyl acrylate, bis(3,4-epoxy-6-methylcyclohexyl methyl) adipate, and 3,4-epoxy-6-methylcyclohexylmethyl-3,4 - epoxy-6-methylcyclohexane-carboxylate.

#### References Cited by the Examiner

##### UNITED STATES PATENTS

|           |         |                  |       |           |
|-----------|---------|------------------|-------|-----------|
| 2,872,427 | 2/1959  | Schroeder        | ----- | 117—145 X |
| 2,909,449 | 10/1959 | Banigan          | ----- | 117—145   |
| 2,949,438 | 8/1960  | Hicks            | ----- | 260—23    |
| 3,008,914 | 11/1961 | Fry              | ----- | 260—837 X |
| 3,054,428 | 9/1962  | Crawford         | ----- | 161—184 X |
| 3,207,718 | 9/1965  | Zimmerman et al. | ----- | 260—29.6  |

20 EARL M. BERGERT, *Primary Examiner*.

HAROLD ANSHER, *Examiner*.